

# United States Patent Office

2,742,413

Patented Apr. 17, 1956

1

2,742,413

## BRIGHT COPPER PLATING BATH

Rolf Cransberg and Hendricus Andreas Van Oosterhout, Loosdrecht, Netherlands, assignors to N. V. Metallic Industry, Loosdrecht, Netherlands, a limited liability company of the Netherlands

No Drawing. Application April 13, 1953,  
Serial No. 348,581

Claims priority, application Netherlands July 5, 1952

9 Claims. (Cl. 204—52)

The electrolytic deposition of copper is an operation which is applied very frequently in the metal industry and is carried out either to embellish the surface of the treated objects or to increase the corrosion resistance thereof, while the electro-deposited copper also serves as a base for a further treatment such as the electrolytic deposition of nickel. In practice high demands are made on the appearance of the treated objects so that these up till now had to be ground and polished in an earlier or later stage of the treatment which entails a number of operations, of which the cost connected therewith form a great part of the total cost of the surface treatment, the electrolytic deposition of copper forms a part of.

Most electrolytic baths have the property that they do not fill up unevennesses in the metal surface such as scratches and the like but rather accentuate them, and especially the baths for the electro-deposition of bright metal layers, from which a very fine crystalline metal deposit is precipitated, have the property that they, besides covering the uneven metal surface with a bright metal layer, also cover the unevennesses only with a thin layer, due to which the latter, although lustrous, remain visible in an undiminished degree.

It has now been found that the acid copper bath in so far makes a favorable exception on the baths, that it has some filling action, in other words, partially fills up gaps, pits and other unevennesses in the surface so that one aimed at improving the filling action of the copper bath, while maintaining other favorable properties such as the capacity to deposit a soft coating on the metal, etc.

It has been proposed to meet the above-described need by adding an organic substance to the copper bath. It is known e. g. from the U. S. P. 1,903,860 to add thiourea or a water-soluble derivative of thiourea, such as methylthiourea, to metal baths. It has been found, however, that the copper coating which is precipitated from the copper baths thus prepared, is very hard, so that it easily springs off on bending and moreover has a very small lustrous range which is considered as a very serious drawback of these baths. Moreover, the action of a copper bath containing exclusively thiourea as an organic compound decreases very soon.

It has now been found that a soft copper layer is obtained if the combination of thiourea or a water-soluble derivative of thiourea and a water-soluble heterocyclic nitrogen compound is added to an acid copper bath. The bath thus prepared displays moreover an excellent filling capacity and has a wide lustrous range.

According to the invention objects, particularly metal objects, are electrolytically provided with a copper deposit with the aid of an acid bath by using a bath containing the combination of a water-soluble derivative of thiourea and a water-soluble heterocyclic nitrogen compound.

The invention extends to the preparation of an acid copper bath containing the combination of thiourea or a

2

water-soluble derivative of thiourea and a water-soluble heterocyclic nitrogen compound, as well as to objects electrolytically provided with a copper layer with the aid of the bath.

5 Of the water-soluble heterocyclic nitrogen compounds which are used in combination with thiourea or a water-soluble derivative of thiourea in the acid copper bath, compounds of the xanthine group, particularly the methyl homologues, such as caffeine (1,3,7-trimethylxanthine), 10 theophylline (1,3-dimethylxanthine) and theobromine (3,7-dimethylxanthine) are preferred, as well as hexamethylene tetramine, morpholine and pyridine, as well as the ring systems, containing the pyridine nucleus, such as quinoline.

15 Of the water-soluble thiourea derivatives which are added to the bath in combination with the heterocyclic nitrogen compounds allyl thiourea is preferred as well as acetylthiourea, while the thiourea itself, if possible, still exceeds in activity these two above-mentioned 20 thiourea derivatives.

The invention is elucidated by the following examples:

### Example I

25 An acid copper bath of the following composition was prepared:

|                                |        |     |
|--------------------------------|--------|-----|
| CuSO <sub>4</sub> ·5 aq.       | g./l.  | 200 |
| H <sub>2</sub> SO <sub>4</sub> | g./l.  | 15  |
| 30 Thiourea                    | mg./l. | 10  |
| Pyridine                       | mg./l. | 40  |

This bath was brought at a temperature of 30° C. and was kept in motion by blowing in a current of air. The anode was of copper. As the cathode a 50 cm. long iron tube with a diameter of 3.5 cm. and a wall thickness of 2 mm. was connected after it having been subjected as a short pretreatment in a cyanide copper bath to a so-called "copper strike" in which a copper layer of very slight thickness was deposited on the outer wall and on a small part of the inner surface adjacent to the ends. The cathode current density of the main treatment in the acid copper bath according to the invention was adjusted to 8 a./dm.<sup>2</sup> and in 20 minutes 32 $\mu$  of copper was deposited on the tube. The copper layer was soft and lustrous, and the numerous unevennesses originally present on the surface of the tube, had substantially disappeared after the electro-deposition of the copper in the above-described bath.

### Example II

An acid copper bath of the following composition was prepared:

|                                |        |     |
|--------------------------------|--------|-----|
| CuSO <sub>4</sub> ·5 aq.       | g./l.  | 250 |
| H <sub>2</sub> SO <sub>4</sub> | g./l.  | 20  |
| Ammonium sulphate              | g./l.  | 20  |
| Acetyl thiourea                | mg./l. | 20  |
| 60 Caffeine                    | mg./l. | 50  |

In this bath an iron plate of 4.5 x 25 dm. was provided with a copper layer at a bath temperature of 25° C. and a cathode current density of 6 a./dm.<sup>2</sup>. The motion of the bath was maintained as in Example I. After 30 minutes a soft lustrous copper layer with a thickness of 30 $\mu$  was deposited on the surfaces of the sheet. The unevennesses originally present in the surface of the sheet were much less deep after the deposition of the copper. Also this iron object was subjected to a "copper strike" beforehand.

## Example III

An acid copper bath of the following composition was prepared:

|                         |        |     |
|-------------------------|--------|-----|
| Copper fluoborate       | g./l.  | 400 |
| Fluoboric acid          | g./l.  | 50  |
| Thiourea                | mg./l. | 12  |
| Hexamethylene tetramine | mg./l. | 800 |

A brass cylinder of 3 dm. length and a diameter of 2.7 cm. was provided with a copper layer in this bath at 28° C. and a motion of, the bath as in Example I during 45 minutes at a cathode current density of 5.5 a./dm.<sup>2</sup>. The thickness of the soft and lustrous copper layer obtained was 50 $\mu$ . After the deposition of the copper no trace of unevennesses could be seen. The original surface displayed scratches which were just perceptible to the naked eye.

## Example IV

An acid copper bath of the following composition was prepared:

|                                |        |     |
|--------------------------------|--------|-----|
| CuSO <sub>4</sub> .5 aq        | g./l.  | 250 |
| H <sub>2</sub> SO <sub>4</sub> | g./l.  | 20  |
| Ammonium sulphate              | g./l.  | 20  |
| Allyl thiourea                 | mg./l. | 20  |
| Morpholine                     | mg./l. | 45  |

A number of small iron plates of 6 x 6 cm. (thickness 0.2 cm.) which had been ground with emery 00 beforehand were provided with a copper layer during 40 minutes at 26° C. in the above-mentioned bath which was kept in motion with air. The cathode current density amounted to 6 a./dm.<sup>2</sup> and the duration of the treatment was 35 minutes. The thickness of the layer was 42 $\mu$ ,

but it is more important that nothing could be seen anymore of the grinding scratches originally present.

What is claimed is:

1. A bright copper plating bath comprising copper sulfate, sulfuric acid, a brightener in proportion of 5 to 50 mg. per liter of solution, said brightener being selected from the group consisting of thiourea, allylthiourea and acetylthiourea, and a filler selected from the group consisting of xanthine and its methyl homologues, hexamethylene tetramine, pyridine and morpholine.
2. A bath according to claim 1, wherein said brightener is thiourea.
3. A bath according to claim 1, wherein said brightener is allylthiourea.
- 15 4. A bath according to claim 1, wherein said brightener is acetylthiourea.
5. A bath according to claim 1, wherein said filler is xanthine.
- 10 6. A bath according to claim 1, wherein said filler is caffeine.
7. A bath according to claim 1, wherein said filler is theobromine.
8. A bath according to claim 1, wherein said filler is theophylline.
- 20 9. A bath according to claim 1, wherein said filler is hexamethylene tetramine.

## References Cited in the file of this patent

## UNITED STATES PATENTS

|           |        |               |
|-----------|--------|---------------|
| 2,391,289 | Beaver | Dec. 18, 1945 |
| 2,700,020 | Pierce | Jan. 18, 1955 |

## FOREIGN PATENTS

|         |        |               |
|---------|--------|---------------|
| 461,186 | Canada | Nov. 22, 1949 |
|---------|--------|---------------|